# EUROPEAN PATENT SPECIFICATION

(11) **EP 0 165 350 B1**
(45) Date of publication and mention of the grant of the patent: **11.01.1989**
(21) Application number: 84304234.2
(22) Date of filing: 22.06.1984
(51) Int. Cl.: C10L 1/32

(54) **Process for producing a high concentration coal-water slurry**
Verfahren zur Herstellung einer Kohle-Wassersuspension mit hohem Kohlegehalt
Procédé de préparation d'une suspension eau-charbon à haute concentration en charbon

(43) Date of publication of application: 27.12.1985
(73) Proprietor: BABCOCK-HITACHI KABUSHIKI KAISHA, Tokyo 100 (JP)
(72) Inventor: Kikkawa, Hirofumi, c/o Kure Research Laboratory, Kure-shi, Hiroshima-ken (JP)
(74) Representative: Pendlebury, Anthony

(56) References cited:
- EP-A- 0 130 849
- WO-A-81/01152
- US-A- 3 762 887

## Description

This invention relates to a coal-water slurry, and more particularly it relates to a process for producing a coal-water slurry having a good stability, a high coal concentration and a low viscosity with minimal settlings.

Recently coal has come to be actively used in place of petroleum mainly at thermal power stations. However, coal in the form of solid fuel is difficult to handle; hance a large transport cost is required which is a great influence on the cost of coal itself. Thus techniques by which coal is slurried to make it possible to handle coal in the form of fluid have been energetically developed. One of the products thus developed is a mixture of heavy oil with coal (Coal and Oil Mixtures, hereinafter referred to as "COM"). In the case of COM, however, the ratio by weight of heavy oil to coal is about 1:1; thus COM cannot be regarded as a oil-free fuel and also its merit in respect of cost is small. Further, methacoal in the form of a mixture of methanol with coal also has a high cost; hence it has not yet been practically used.

On the other hand, CWM in the form of a mixture of coal with water (CWM: abbreviation of Coal-Water Mixtures) is sufficiently practical in respect of cost; hence it has recently been greatly noted. However, a problem raised in the combustion of CWM is water content in CWM. Even as far as its combustion efficiency is concerned, naturally the lower the water content, the better the efficiency, and in the case of direct combustion, a water content of 30% or less is preferred. However, the lower the water content, the higher the viscosity of CWM; this raises a problem that when it is transported by way of pipeline or the like, the pressure loss increases.

Further, when CWM is practically used, a problem of storage is also raised. When CWM is stored in a usual tank, it is necessary for it to have a superior stability, but since CWM consists of coal particles and water, it is preferred to reduce their particle diameter, in order to inhibit coal particles from settling as much as possible. However, there is a tendency that when the particle diameter is reduced, the viscosity increases.

In order to overcome such drawbacks, it has been attempted to adjust the particle diameter distribution of coal particles to thereby prepare a CWM of the so-called "good stability" having a high coal concentration and a low viscosity with minimal settlings. However, coal particles are not completely spherical, and also the method of measuring the particle diameter of coal particles are various as follows: a method by means of sieves, a settling method represented by the "Andreasen Pipette", a method of analyzing the particle shapes by way of photographs of SEM (Scanning Electron Microscope) to calculate their representative diameter, etc. Thus, the definition of the particle diameter also varies depending on the measurement methods. This causes errors in adjusting the particle diameter distribution, and it becomes difficult to produce a CWM having a high coal concentration, a low viscosity and a good stability.

EP-A-0130849 discloses a process for producing a coal-water slurry having a low viscosity and a good stability, even in a high coal concentration, the process comprising feeding coal to a wet mill and grinding it therein, the coal which is fed to the wet mill being divided in a multi-stage manner.

Now, the present inventors have considered that this problem might be solved by adjusting the particle diameter distribution according to a method of measuring the particle diameter distribution regarded as most adequate, and have made extensive research. As a result, we have succeeded in obtaining the objective CWM having a high coal concentration, a low viscosity and a good stability.

The present invention aims to provide a process for producing a coal-water slurry having a high coal concentration, a low viscosity and a good stability.

A process for producing a coal-water slurry having coal particles dispersed in water, which process comprises causing the slurry to have a composition of coal particles, so that when the coal particles are divided into 8 fractions (F₁, F₂, - - - and F_{B}), each having a particle diameter range listed below, ((from D_{L}/4 to D_{L}), (from Dd42 to less than Dd4), - - - (from D_{L}/4⁷ to 0), wherein D_{L} represents the maximum particle diameter of the coal particles), then the proportions by weight of the coal particles contained in the respective fractions, relative to the total weight of the coal particles contained in the slurry fall within the following ranges of numerical values:

characterised in that at least one kind of anionic dispersant selected from the group consisting of naphthalenesulfonic acid, orthophosphoric acid, polyphosphoric acids represented by Hₙ₊₂PₙO₂ₙ₊₁ (n?21 or HₙPₙO₂ₙ (n≧3), tartaric acid, oxalic acid, citric acid, ethylenediamine tetraacetate, ligninsulfonic acid, salts and condensates of the foregoing, tannins including quebracho-tannin and metal salts of carboxymethylcellulose, is added to the slurry, as a dispersant for coal particles in an amount of 3% by weight or less based on the coal weight, and/or at least one kind of pH-adjustor selected from the group consisting of sodium hydroxide, potassium hydroxide, barium hydroxide and sodium carbonate is added to the slurry as a pH-adjustor for rendering the pH value of the slurry 7 or more, in an amount of 3% or less based on the coal weight.

Embodiments of the present invention will now be described by way of example only with reference to the accompanying drawings, in which:
Figure 1 shows a chart illustrating the particle sizes of low viscosity slurries and cumulative particles diameter distributions thereof when produced in accordance with the present invention.
Figure 2 shows a bar chart illustrating particle diameters and proportions by weight of the respective fractions.
Figure 3 shows a diagram illustrating the relationship between particle diameter distributions and slurry viscosities.
Figure 4 shows a chart illustrating the relationship between particle diameter distributions and stability.
Figure 5 shows a chart illustrating the relationship between the amount of dispersant added and viscosity.
Figure 6 shows a chart illustrating the relationship between pH and viscosity.
Figure 7 shows a chart illustrating the relationship between the amount of ultrafine particles of 0.05 pm or less added and stability.
Figure 8 shows a view of piping system illustrating an embodiment of an apparatus for producing CWM.
Figures 9 and 10 each show a chart illustrating the particle diameter of slurry produced by the apparatus of Figure 8 and cumulative sieve pass proportion by weight.

The present invention will be described referring to the accompanying drawings.

Coal is ground in wet or dry manner by means of a mill and a part of the resulting particles is taken to measure their particle diameter distribution. In measuring the particle diameter distribution, it was considered that the weight proportion of finely divided particles had a great influence upon the viscosity and the stability relative to the setting of the slurry. Thus in an example, the particles were divided into the following 8 fractions (each a constituent part as a group), and the respective fractions were each sieved by a sieve most adequate thereto (e.g. sieve according to JIS standards or millipore filter having the particle diameter well adjusted) to measure the weight of the fraction.

In the following list, D_{L} represents the maximum particle diameter of particles. F₁ to Fₐ represent symbols of the respective fractions.

In the present invention, particles were divided into 8 fractions for measurement, but the number of fractions is not always limited to 8, but practically it may be from 5 to 15 unless the distribution of the particle sizes changes.

More than one kind of coal or coal slurry were mixed so that the constituent proportions by weight of F₁ to F₈ might have a certain value, respectively, and if necessary, water was added for adjusting the water content, to study their viscosities. In this case, if the maximum particle diameter D_{L} is too large, the amount of unburned matter at the time of combustion increases, while if it is too small, the slurry viscosity increases; hence the maximum particle diameter D_{L} was made from 44 to 420 pm.

Further, a certain kind of coal was chosen and the proportions of fractions were varied to study the influence upon viscosity. Further, when proportions of fractions exhibiting a relatively low viscosity were converted into cumulative distributions, a tendency was found. Figure 1 shows a chart illustrating the relationship between the particle diameter and the cumulative sieve pass weight proportion in the case where three kinds of slurries (No. 1 to No. 3) were prepared from coal A (bituminous coal, ash content 9.5%). There are shown cumulative particle diameter distributions in the case of a coal concentration of 70% and 1000 mPas (cP) or less. In this case, the maximum particle diameter D_{L} is 297 µm and only distributions of particle sizes of 1 pm or larger are shown. Further, the slurry viscosity refers to numerical values obtained when an inner cylinder-rotation type viscometer was rotated at a shear rate of 90 sec-1 for 5 minutes. It is seen from Figure 1 that the proportions in the case of 1 µm or more each constitute a nearly straight line. Further, when the cumulative sieve weight proportion U(D)% is 100% at D=D_{L}, Dₛ (minimum particle diameter) at which U(D)=0% should be present. Thus, we propose the following equations (1) and (2) as those indicating a particle diameter distribution mode of coal particles contained in a slurry exhibiting a low viscosity at a high coal concentration: wherein q represents an index.

In both the equation (1) and (2), when D=D_{L}, U(D)=100%, and when D=Dₛ, U(D)=0%. That is, these equations correspond well to practical particle size distributions.

If Dₛ=0 in the equation (1) and (2), the equations both give the following equation (3):

This equation (3) corresponds to Andreasen's equation which has been known as a particle diameter distribution equation giving the closest packing for powder of a continuous particle size system. As to this Andreasen's equation, studies were made in the past, and it was confirmed that when q=from 0.35 to 0.40, the percentage packing attains the maximum. The percentage packing, however, varies depending on particle shapes, and as to the systematic relationship between the q value and the slurry viscosity and stability of coal-water slurry, no study has ever been made. Further, Andreasen's equation is a distribution equation in the case where particles having an infinitesimal particle diameter were presumed, but the equation cannot be, as it is, applied to a practical coal-water slurry. In contrast the present inventors confirmed that the equation (1) and (2) correspond well to practical distributions.

Figure 2 shows the weight proportions of the respective fractions in the case where D_{L}=297 µm, Dₛ=0.01 µm and q=0.3 in the equations (1) and (2). In this case, in order to compare the particle diameters more strictly, particles were divided into the following 15 fractions (dotted lines in Figure 2 indicate the case of the equation (2) and solid lines therein indicate the case of the equation (1)):

It is seen that the case of the equation (1) is different from that of the equation (2) in that the proportion of finely divided particles is higher and there are minimum points F₁₃ and F₁₄ where the weight proportion becomes minimum.

Thus, the present inventors varied the values of D_{L}, Dₛ and q in the equations (1) and (2) to study their influences upon the viscosity and stability of slurry, whereby many findings could be obtained.

From these findings, coal-water slurry of the present invention is preferably composed so that diameter distribution of coal particles having particle diameters in the range of from 1,000 µm to 0.005 pm substantially satisfies the following equation and the following ranges of numeral values:
(2) D_{L}=from 44 to 1,000 pm
(3) Dₛ=from 0.005 to 0.1 µm
(4) q=from 0.25 to 0.50
wherein D represents a particle diameter of coal particles; D_{L}, the maximum particle diameter thereof; D_{S}, the minimum particle diameter thereof; and q, an index.

Further, the slurry is preferably composed so that coal particles of 1 pm or less can be present in an amount of from 5 to 46% by weight and those of 0.05 um or less can be present in an amount of 0.5% or more, more preferably 1% or more.

Further, it is preferable that the coal-water slurry has a coal content of 60 to 80% by weight and a viscosity of 5,000 mPas (cP) or less, in terms of numerical values obtained when an inner cylinder-rotation type viscometer is rotated at a shear rate of 90 sec⁻¹ for 5 minutes.

A coal-water slurry when produced by the process of the present invention includes at least one kind of anionic dispersant selected from the group consisting of naphthalenesulfonic acid, orthophosphoric acid, polyphosphoric acids represented by Hₙ₊₂PₙO₂ₙ₊₁ (n≧2) or HₙPₙO₂ₙ (n≧3), tartaric acid, oxalic acid, citric acid, ethylenediamine tetraacetate, ligninsulfonic acid, salts or condensates of the foregoing, tannins including quebracho-tannin and metal salts of carboxymethylcellulose, as a dispersant for coal particles in an amount of 3% by weight, or less, preferably 1.5% or less, based on the weight of the coal, and/or at least one kind of pH-adjustor selected from the group consisting of sodium hydroxide, potassium hydroxide, barium hydroxide and sodium carbonate may be added to the slurry as a pH-adjustor for rendering the pH value of the slurry 7 or more, in an amount of 3% or less, preferably 1.5% or less, based on the coal weight.

The present invention will be described in more detail by way of Examples.

### Example 1

With coal A (bituminous coal, ash content 9.5%), the proportions of the respective fractions were adjusted according to the above-mentioned method to prepare 20 kinds of coal samples having particle diameter distributions corresponding to D_{L}=297 pm and 149 µm, Dₛ=0.01 µm and q=0.15, 0.20, 0.25, 0.30, 0.35, 0.40, 0.45, 0.50, 0.55 and 0.60 in the equation (1), followed by preparing a slurry having a coal concentration of 72% by adjusting the water content of the respective samples, thereafter adding a poly-sodium naphthalenesulfonate as dispersant in an amount of 0.5% based on the coal weight and sodium hydroxide as pH adjustor in an amount of 0.1% based thereon and measuring their slurry viscosities. The results are shown in Figure 3. It was observed that the viscosities became minimum at q=from 0.40 to 0.45 irrespective of D.

The same studies were made as to the equation (2) to similarly give the minimum viscosities at q=from 0.40 to 0.45. Further, it was observed that the viscosity values, too, accorded nearly with the above in the case of the same values of D_{L}, Dₛ and q.

Further, the same studies were made on other kinds of coals to give the minimum viscosities at q=from 0.40 to 0.50.

### Example 2

With the same slurries as in Example 1, their stabilities were studied. Each of the slurries was placed in a 500 ml graduated cylinder up to a depth of 170 mm, followed by allowing a glass stick of 5 mm in diameter and 10 g in weight to penetrate thereinto only by its self weight to observe the change in the penetration time during which the stick reached the bottom of the cylinder. Figure 4 shows the relationship between the penetration time at the time when 30 days lapsed after preparation of the slurries (the penetration time just after the preparation being made), and the q value. Namely Figure 4 shows comparison of stabilities as to the slurries having viscosities shown in Figure 3 and D_{L}=297 pm. The penetration time became minimum at q=from 0.25 to 0.35, and it is seen that the penetration time is shorter and the stability is superior in the case of the equation (1) as compared with those in the case of the equation (2).

Other kinds of coals were studied varying C_{L}, etc. to obtain similar results.

It was found through Examples 1 and 2 that slurries according to the equation (1) were superior in stability to those according to the equation (2) and they exhibited equal values as to viscosity. Further it was found that in view of viscosity and stability, particle diameter distributions at q=from 0.25 to 0.50 in the equation (1) were preferable.

### Example 3

With coal B (bituminous coal, ash content 13.6%), Example 1 was repeated to prepare a slurry having a particle diameter distribution corresponding to D_{L}=297 µm, Dₛ=0.01 pm and q=0.40 in the equation (1) and a coal concentration of 70%. A condensate of sodium naphthalinesulfonate as dispersant was added to the slurry to observe the relationship between its amounts added and the slurry viscosities. The results are shown in Figure 5. In this case, the addition amounts are values based on the coal weight, and sodium hydroxide was added as pH adjustor in an amount of 0.1% based on the coal weight.

The viscosities became minimum in an addition amount of 0.5% of the dispersant, and more amounts resulted in an adverse effect.

Other kinds of coals were similarly studied, and the viscosities became minimum in addition amounts of from 0.2 to 1.2%. When other anionic dispersants were added, slurries having a minimum viscosity were similarly obtained in addition amounts of from 0.1 to 1.5%.

### Example 4

With coal B (bituminous coal, ash content 13.6%), the same slurry as in Example 3 was prepared, followed by varying the amount of sodium hydroxide added, in a fixed amount of 0.5% of a condensate of sodium naphthalenesulfonate being added, to adjust the pH of slurry to thereby study the influence of pH upon slurry viscosity. The results are shown in Figure 6. Up to pH 8, the higher the pH, the lower the slurry viscosity, and at higher pHs, the viscosity is almost unchanged. Taking into consideration the amount of sodium hydroxide consumed and corrosion of material, a pH of from 7 to 9 is preferred. In the case of coal, although the pH of slurry prepared therefrom varies depending on the kind of coal and the oxidation degree of its surface, the amount of sodium hydroxide added, necessary for adjusting the pH from 7 to 9, is from 0 to 1.0% based on the weight of coal.

### Example 5

Ultrafine particles having passed through a millipore filter of 0.05 pm were further added to a slurry of coal B having a particle diameter distribution expressed by the equation (1) and corresponding to D_{L}=297 µm, Dₛ=0.01 µm and q=0.40, to study the influence of the ultrafine particles upon the stability of the slurry. The results are shown in Figure 7. In this figure, the penetration time of the ordinate axis refers to a ratio of the penetration time in 30 days after preparation of slurry to that just after the preparation, and the amount of ultrafine particles added refers to a proportion thereof based on the total weight of coal after the addition.

The stability is best in an amount of the ultrafine particles added of 3%, and it is seen that particles of 0.05 µm or less contributed to the slurry stability. Studies were carried out varying the particle diameter distribution and the kind of coal. As a result it was found that the viscosity was unchanged when the weight of particles of 0.05 µm or less effective for improving the slurry stability fell within the range of from 0.5 to 6.5% (preferably from 1.0 to 4.0%). Further, it was found that this tendency was unchanged even when the kind of coal, its concentration and D_{L} were varied.

### Example 6

With coal A (bituminous coal, ash content 9.5%), a process for preparing a slurry having a particle diameter distribution corresponding to the equations (1) and (2), by means of a tube ball mill was studied. The apparatus and flow in this case are shown in Figure 8. Coal stored in a hopper 1 was fed into a mill 3 through a feeder 2, and at the same time, water and additives were fed into the mill through a feed pipe 4. At that time, conditions were established so as to give a coal concentration of 70% and average retention times of coal in the mill, of 90 minutes and 120 minutes, and when a stationary state was attained, the resulting slurries were taken to observe their particle diameter distributions. The results are shown in Figure 9. It is seen that the slurries had particle diameter distributions corresponding to D_{L}=420 µm, Dₛ=0.04 µm and q=0.40, and D_{L}=300 pm, Dₛ=0.01 pm and q=0.40 in the equation (2).

Next, 10% of the slurry of the average retention time of 120 minutes discharged from the exit of the mill was returned to the inlet of the mill and again ground. When a stationary state was attained, particle diameters were measured to give a particle diameter distribution corresponding to D_{L}=300 µm, Dₛ=0.01 µm and q=₀.40 in the equation (1). See Figure 10.

Other kinds of coals were similarly studied. As a result, it was found that in order to prepare a slurry having a particle diameter distribution according to the-equation (1) and a good stability, it was impossible to achieve the object merely by adjusting the retention time in the mill, but a process of recycling from 10 to 50% of the product slurry (i.e. recycling feed) was effective.

In view of the above-mentioned Examples, it has been found that in order to obtain a CWM having a high coal concentration, a low viscosity and a good stability, if a strict and systematic control of the particle diameter distribution is conducted by means of sieves and the particle diameter distribution is caused to comply with the following equation, then the viscosity and stability of the resulting slurry becomes optimum: wherein
q=from 0.25 to 0.50
D_{L}=from 44 to 420 pm
Dₛ=from 0.005 to 0.1 µm

Further it has been found that when finely divided particles of 0.05 pm or less are present in an amount of from 0.5 to 6.5% (preferably from 1.0 to 4.0%), the slurry stability becomes optimum.

Furthermore it has been found that the amount of the dispersant added is optimum in a range of from 0.1 to 1.5% and it is preferred to add a pH adjustor so as to give a pH of from 7 to 9.

When this invention is conducted, there is exhibited an effectiveness of rendering a mixture of water with powdered coal, a water-coal slurry having a high coal concentration, a low viscosity and a good stability with settlings being formed only with difficulty.

## Claims

1. A process for producing a coal-water slurry having coal particles dispersed in water, which process comprises causing the slurry to have a composition of coal particles, so that when the coal particles are divided into 8 fractions (F₁, F₂, ...and F₈), each having a particle diameter range listed below, ((from D_{L}/4 to D_{L}), (from D_{L}/4² to less than D_{L}/4), ... (from D_{L}/4⁷ to 0), wherein D_{L} represents the maximum particle diameter of the coal particles), then the proportions by weight of the coal particles contained in the respective fractions, relative to the total weight of the coal particles contained in the slurry fall within the following ranges of numerical values:
characterised in that at least one kind of anionic dispersant selected from the group consisting of naphthalenesulfonic acid, orthophosphoric acid, polyphosphoric acids represented by Hₙ₊₂PₙO₂ₙ₊₁ (n≧2) or HₙPₙO₂ₙ (n≧3), tartaric acid, oxalic acid, citric acid, ethylenediamine tetraacetate, ligninsulfonic acid, salts and condensates of the foregoing, tannins including quebracho-tannin and metal salts of carboxymethylcellulose, is added to the slurry, as a dispersant for coal particles in an amount of 3% by weight or less based on the coal weight, and/or at least one kind of pH-adjustor selected from the group consisting of sodium hydroxide, potassium hydroxide, barium hydroxide and sodium carbonate is added to the slurry as a pH-adjustor for rendering the pH value of the slurry 7 or more, in an amount of 3% or less based on the coal weight.

2. A process according to Claim 1, wherein the particle diameter distribution of coal particles having particle diameters in the range of from 1,000 pm to 0.005 pm substantially satisfies the following equation and the following ranges of numerical values:
(2) D_{L}=from 44 to 1,000 µm
(3) Dₛ=from 0.005 to 0.1 pm
(4) q=from 0.25 to 0.50
wherein D represents a particle diameter of coal particles; D_{L}, the maximum particle diameter thereof; D_{S}, the minimum particle diameter thereof; and q, an index.

3. A process according to Claim 1, or Claim 2, wherein the coal particles in the slurry are composed so that coal particles of 1 µm or less can be present in an amount of from 5 to 46% by weight and those of 0.05 µm or less can be present in an amount of 0.5% or more.

4. A process according to any one of Claims 1 to 3, wherein the slurry has a coal content of from 60 to 80% by weight and a viscosity of 5,000 mPas (cP) or less, in terms of numerical values obtained when an inner cylinder-rotation type viscometer is rotated at a shear rate of 90 sec⁻¹ for 5 minutes.

5. A coal-water slurry having a composition of coal particles, so that when the coal particles are divided into 8 fractions (F₁, F₂, - - - and F₈), each having a particle diameter range listed below, ((from D_{L}/4 to D_{L}), (from D_{L}/4² to less than D_{L}/4), ... (from D_{L}/4⁷ to 0), wherein DL represents the maximum particles diameter of the coal particles), then the proportions by weight of the coal particles contained in the- respective fractions, relative to the total weight of the coal particles contained in the slurry fall within the following ranges of numerical values:
characterised in that at least one kind of anionic dispersant selected from the group consisting of naphthalenesulfonic acid, orthophosphoric acid, polyphosphoric acids represented by Hₙ₊₂PₙO₂ₙ₊₁ (n≧2) or HₙPₙO₂ₙ (n≧3), tartaric acid, oxalic acid, citric acid, ethylenediamine tetraacetate, ligninsulfonic acid, salts and condensates of the foregoing, tannins including quebracho-tannin and metal salts of carboxymethylcellulose, is comprised in the slurry, as a dispersant for coal particles in an amount of 3% by weight or less based on the coal weight, and/or at least one kind of pH-adjustor selected from the group consisting of sodium hydroxide, potassium hydroxide, barium hydroxide and sodium carbonate is comprised in the slurry as a pH-adjustor for rendering the pH value of the slurry 7 or more, in an amount of 3% or less based on the coal weight.

## Patentansprüche

1. Verfahren zur Herstellung einer Kohlenstaub/Wasser-Trübe, in welcher Kohleteilchen in Wasser dispergiert sind, wobei die Trübe auf eine Zusammensetzung der Kohleteilchen dergestalt gebracht wird, daß dann, wenn die Kohleteilchen in 8 Teilmengen (Fᵢ, F₂, - - - und F₈) eingeteilt werden, von denen jede einen Teilchendurchmesser gemäß untenstehender Liste aufweist, ((von D_{L}/4 bis D_{L}), (von D_{L}/4² bis weniger als D_{L}/4), ... (von D_{L}/4⁷ bis 0), worin D_{L} den maximalen Teilchendurchmesser der Kohleteilchen darstellt), die Gewichtsanteile der in den entsprechenden Teilmengen enthaltenen Kohleteilchen im Verhältnis zum Gesamtgewicht der in der Trübe enthaltenen Kohleteilchen innerhalb folgender Zahlenwertgruppen liegen:
dadurch gekennzeichnet, daß der Trübe mindestens eine Art von anionischen Dispersionsmitteln, ausgewählt aus der Gruppe, welche Naphthalinsulfonsäure, Orthophosphorsäure, Polyphosphorsäuren dargestellt durch Hₙ₊₂PₙO₂ₙ₊₁ (n≧2) oder HₙPₙO₂ₙ (n≧3), Weinsäure, Oxalsäure, Zitronensäure, Äthylendiaminotetraazetat, Ligninsulfonsäure, Salze und Kondensate derselben, Tannine einschließlich Quebrachotannin und Metallsalze von Karboxymethylzellulose umfaßt, als Dispersionsmittel für Kohlenteilchen zugesetzt wird, in einer Menge von 3% im Gewichtsanteil oder weniger, bezogen auf das Kohlegewicht, und/oder daß der Trübe mindestens eine Art von pH-Einstellmittel, ausgewählt aus der Gruppe, welche Natriumhydroxid, Kaliumhydroxid, Bariumhydroxid und Natriumkarbonat umfaßt, als pH-Einstellmittel zugesetzt wird, um den pH-Wert der Trübe auf einen Wert von 7 oder mehr zu bringen, in einer Menge von 3% oder weniger, bezogen auf das Kohlegewicht.

2. Verfahren nach Anspruch 1, dadurch gekennzeichnet, daß die Teilchendurchmesser-Verteilung der Kohleteilchen mit Teilchendurchmessern im Bereich von 1.000 um bis 0,005 µm die nachstehende Gleichung erfüllt und folgenden Zahlenwertbereichen entspricht:
(2) D_{L}=von 44 bis 1.000 um
(3) Dₛ=von 0,005 bis 0,1 µm
(4) q=von 0,25 bis 0,50
worin D den Teilchendurchmesser der Kohleteilchen; D_{L} den maximalen Teilchendurchmesser derselben; Dₛ den kleinsten Teilchendurchmesser derselben und q einen Exponenten darstellt.

3. Verfahren nach Anspruch 1 oder 2, dadurch gekennzeichnet, daß die Kohleteilchen in der Trübe derart zusammengesetzt sind, daß Kohleteilchen von 1 µm oder kleiner in einer Menge von 5 bis 46% im Gewichtsanteil und solche von 0,05 µm oder kleiner in einer Menge von 0,05% oder mehr vorhanden sein können.

4. Verfahren nach einem der Ansprüche 1 bis 3, dadurch gekennzeichnet, daß die Trübe einen Kohlegehalt von 60 bis 80% im Gewichtsanteil und eine Viskosität von 5.000 mPas (cP) oder weniger aufweist, wobei die Zahlenwerte erhalten werden, wenn ein Innenzylinder - Rotationsviskosimeter mit einem Schergefälle von 90 sec⁻¹ 5 Minuten lang gedreht wird.

5. Kohlenstaub/Wasser-Trübe, in welcher Kohleteilchen in Wasser dispergiert sind, wobei die Trübe auf eine Zusammensetzung der Kohleteilchen dergestalt gebracht wird, daß dann, wenn die Kohleteilchen in 8 Teilmengen (Fᵢ, F₂, ... und F₈) eingeteilt werden, von denen jede einen Teilchendurchmesser gemäß untenstehender Liste aufweist, ((von D_{L}/4 bis D_{L}), (von D_{L}/4² bis weniger als D_{L}/4), - - - (von D_{L}/4⁷ bis 0), worin D_{L} den maximalen Teilchendurchmesser der Kohleteilchen darstellt), die Gewichtsanteile der in den entsprechenden Teilmengen enthaltenen Kohleteilchen im Verhältnis zum Gesamtgewicht der in der Trübe enthaltenen Kohleteilchen innerhalb folgender Zahlenwertgruppen liegen:
dadurch gekennzeichnet, daß der Trübe mindestens eine Art von anionischen Dispersionsmitteln, ausgewählt aus der Gruppe, welche Naphthalinsulfonsäure, Orthophosphorsäure, Polyphosphorsäuren dargestellt durch Hₙ₊₂PₙO₂ₙ₊₁ (n≧2) oder HₙPₙO₂ₙ (n≧3), Weinsäure, Oxalsäure, Zitronensäure, Äthylendiaminotetraazetat, Ligninsulfonsäure, Salze und Kondensate derselben, Tannine einschließlich Quebrachotannin und Metallsalze von Karboxymethylzellulose umfaßt, als Dispersionsmittel für Kohleteilchen zugesetzt wird, in einer Menge von 3% im Gewichtsanteil oder weniger, bezogen auf das Kohlegewicht, und/oder daß der Trübe mindestens eine Art von pH-Einstellmittel, ausgewählt aus der Gruppe, welche Natriumhydroxid, Kaliumhydroxid, Bariumhydroxid und Natriumkarbonat umfaßt, als pH-Einstellmittel zugesetzt wird, um den pH-Wert der Trübe auf einen Wert von 7 oder mehr zu bringen, in einer Menge von 3% oder weniger, bezogen auf das Kohlegewicht.

## Revendications

1. Procédé de préparation d'une suspension charbon-eau, constituée de particules de charbon en dispersion dans de l'eau, lequel procédé consiste à faire en sorte que la suspension ait une composition de particules de charbon telle que, quand les particules de charbon sont subdivisées en 8 fractions (Fᵢ, F₂, ... et F₈), chacune d'entre elles correspondant à l'intervalle granulométrique indiqué ci-dessous ((de D_{L}/4 à D_{L}), (de D_{L}/4² à moins de D_{L}/4), ... (de D_{L}/4⁷ à 0), où D_{L} représente le diamètre maximum des particules de charbon), les proportions pondérales des particules de charbon contenues dans les fractions respectives, par rapport au poids total des particules de charbon contenues dans la suspension, tombent dans les intervalles suivants en valeurs numériques:
caractérisé en ce qu'on ajoute à la suspension au moins un type d'un dispersant anionique choisi dans le groupe comprenant l'acide naphtalènesulfonique, l'acide orthophosphorique, les acides poly- phosphoriques représentés par Hₙ₊₂PₙO₂ₙ₊₁ (n≥21) ou HₙPₙO₂ₙ (n≥3), l'acide tartrique, l'acide oxalique, l'acide citrique, un éthylènediaminetétraacétate, l'acide ligninesulfonique, les sels et produits de condensation des composés ci-dessus, les tannins, y compris le tannin de québracho et sels métalliques de la carboxyméthylcellulose, et ce en tant que dispersants des particules de charbon, en une quantité de 3% en poids ou moins par rapport au poids du charbon, et/ou qu'on ajoute à la suspension au moins un type d'un régulateur de pH choisi dans le groupe comprenant l'hydroxyde de sodium, l'hydroxyde de potassium, l'hydroxyde de baryum et le carbonate de sodium, en tant que régulateurs de pH pour amener le pH de la suspension à 7 ou plus, en une quantité de 3% ou moins par rapport au poids du charbon.

2. Procédé selon la revendication 1, dans lequel la répartition granulométrique des particules de charbon ayant des diamètres de particules compris entre 1000 et 0,005 pm satisfait essentiellement à l'équation suivante et aux intervalles suivants de valeurs numériques:
(1) U(D)=[(D-Dₛ)/(D_{L}-Dₛ)]^{q}×100
(2) D_{L}=de 44 à 1000 pm
(3) Dₛ=de 0,005 à 0,1 pm
(4) q=_{d}e 0,25 à 0,50
où D représente le diamètre des particules de charbon; D_{L} le diamètre maximum de ces particules; Dₛ le diamètre minimal de ces particules; et q est un indice.

3. Procédé selon la revendication 1 ou la revendication 2, dans lequel les particules de charbon se trouvant dans la suspension sont constituées de façon que les particules de charbon de 1 µm ou moins puissent être présentes en une quantité de 5 à 46% en poids, et celles de 0,05 µm ou moins puissent être présentes en une quantité de 0,5% ou plus.

4. Procédé selon l'une quelconque des revendications 1 à 3, dans lequel la suspension a une teneur en charbon de 60 à 80% en poids et une viscosité de 5000 mPa . s (cP) ou moins, exprimées en les valeurs numériques obtenues quand on fait tourner à une vitesse de cisaillement de 90 s⁻¹ pendant 5 minutes un viscosimètre du type à rotation par cylindre interne.

5. Suspension eau-charbon ayant une composition de particules de charbon telle que, quand les particules de charbon sont subdivisées en 8 fractions (F₁, F₂, ... et F₈), chacune d'entre elles ayant l'intervalle granulométrique indiqué ci-dessous ((de D_{L}/4 à D_{L}), (de D_{L}/4² à moins de D_{L}/4), ... (de D_{L}/4⁷ à 0), où D_{L} représente le diamètre maximum des particules de charbon), les proportions pondérales des particules de charbon contenues dans les fractions respectives, par rapport au poids total des particules de charbon contenues dans la suspension, tombent dans les intervalles suivants, en valeurs- numériques:
caractérisé en ce qu'on ajoute à la suspension au moins un type d'un dispersant anionique choisi dans le groupe comprenant l'acide naphtalènesulfonique, l'acide orthophosphorique, les acides poly- phosphoriques représentés par Hₙ₊₂PₙO₂ₙ₊₁ (n≥2) ou HₙPₙO₂ₙ (n≥3), l'acide tartrique, l'acide oxalique, l'acide citrique, en éthylènediaminetétracétate, l'acide ligninesulfonique, les sels et produits de condensation des composés ci-dessus, les tannins, y compris le tannin de québracho et sels métalliques de la carboxyméthylcellulose, et ce en tant que dispersants des particules de charbon, en une quantité de 3% en poids ou moins par rapport au poids du charbon, et/ou qu'on ajoute à la suspension au moins un type d'un régulateur de pH choisi dans le groupe comprenant l'hydroxyde de sodium, l'hydroxyde de potassium, l'hydroxyde de baryum et le carbonate de sodium, en tant que régulateurs de pH pour amener le pH de la suspension à 7 ou plus, en une quantité de 3% ou moins par rapport au poids du charbon.
